# EUROPEAN PATENT SPECIFICATION

(11) **EP 0 897 732 B1**
(45) Date of publication and mention of the grant of the patent: **31.12.2008**
(21) Application number: 98306409.8
(22) Date of filing: 11.08.1998
(51) Int. Cl.: A63B 37/00

(54) **Multi-piece solid golf ball**
Mehrteiliger, fester Golfball
Balle de golf solide en plusieurs pièces

(30) Priority: 11.08.1997 JP 22890297
(43) Date of publication of application: 24.02.1999
(73) Proprietor: BRIDGESTONE SPORTS CO., LTD., Tokyo (JP)
(72) Inventor: Yamagishi, Hisashi, Bridgestone Sports Co., Ltd., Chichibu-shi, Saitama-ken (JP); Higuchi, Hiroshi, Bridgestone Sports Co., Ltd., Chichibu-shi, Saitama-ken (JP); Hayashi, Junji, Bridgestone Sports Co., Ltd., Chichibu-shi, Saitama-ken (JP); Kawata, Akira, Bridgestone Sports Co., Ltd., Chichibu-shi, Saitama-ken (JP)
(74) Representative: Whalley, Kevin

(56) References cited:
- GB-A- 2 298 583
- GB-A- 2 301 291
- GB-A- 2 306 118

## Description

### Field of the Invention

This invention relates to a multi-piece sold golf ball having a cover of inner and outer layers and more particularly, to a multi-piece solid golf ball in which cover hardness and dimples are optimised so as to improve flight distance performance.

### Prior Art

Golf balls are generally classified into solid golf balls in which a solid core is enclosed with at least one layer of cover and wound golf balls in which a wound core in the form of a center ball having thread rubber wound thereon is enclosed with a cover. Numerous modifications were heretofore proposed to improve flight distance properties, spin performance, and controllability.

GB231291, for example, discloses a thread-wound golf ball with a controlled number of dimples and dimple volume rate and a specified solid center to show good spin properties and good restitution.

As one example of such proposals, an approach of increasing a spin rate by forming the cover soft or to low hardness falls under the category of the prior art. In particular, improvements in multi-piece solid golf balls are by adjusting the composition and hardness of the thermoplastic resin of which each cover layer is constructed. For example, if it is desired to increase a spin rate, the outer cover layer coming in direct contact with the club face is formed relatively soft in consideration of a friction phenomenon upon impact. Inversely, if it is desired to decrease a spin rate, the outer cover layer is formed relatively hard.

GB2298583 discloses a golf ball comprising a solid core enclosed with a single cover layer of Shore D hardness of at least 60 and a specified dimple volume rate.

US5033750 discloses a golf ball with improved flight distance, wherein a relationship between the diameter and depth of each dimple is optimised among two or more different types of dimples.

However, the multi-piece solid golf balls wherein the outer cover layer is formed relatively soft have the problem that a desired spin rate is not always obtained because the hardness of the inner cover layer in contact with the outer cover layer is not optimized and thus, the deformation process upon impact differs among the respective layers.

Also proposed were techniques of forming the inner cover layer relatively soft in order to increase a spin rate and forming the outer and inner cover layers relatively soft in order to further increase a spin rate. There arises the problem that the trajectory changes in flight to adversely affect the flight distance.

On the other hand, for those golf balls required to have flight distance performance, it is difficult to form dimples suitable for the spin range and restitution which vary with the cover hardness. Golf balls with dimples of one type suffer from the problem that they rise too high or drop to detract from the flight distance performance.

The present invention has been made under the above-mentioned circumstances and its object is to provide a golf ball comprising a solid core enclosed with two inner and outer layers enabling to increase a flight distance.

Making extensive investigations to achieve the above object, we have found in connection with a multi-piece solid golf ball comprising a solid core and a cover of two inner and outer layers surrounding the core, the outer cover layer being formed in the surface with a plurality of dimples, that a spin rate is approximately explained in terms of a product of the Shore D hardness of the inner cover layer multiplied by the Shore D hardness of the outer cover layer. More particularly, a more spin rate is obtained when the product of the Shore D hardnesses of the inner and outer layers has a relatively smaller value. Inversely, a less spin rate is obtained when the same product has a relatively larger value. Accordingly, effective means for taking full advantage of the spin property dependent on the product of the Shore D hardnesses of the inner and outer layers and improving the flight performance of the golf ball is to divide the range of the product into sub-ranges and form dimples so as to satisfy the following two requirements associated with the sub-ranges of the product. More particularly, it has been found effective as a first requirement to specify a proportion V_{R} (%) of the total of the volumes of dimple spaces each defined below a plane circumscribed by the dimple edge to the overall volume of a phantom sphere given on the assumption that the golf ball surface is free of dimples, and as a second requirement to form at least three types of dimples which are different in at least one of a diameter, a depth, and a value V₀ which is the volume of one dimple space defined below a plane circumscribed by the dimple edge divided by the volume of a cylinder whose bottom is the plane and whose height is the maximum depth of the dimple from the bottom. We have also found that to specify the distortion of the solid core and to specify the Shore D hardness of the inner and outer cover layers are more effective. The present invention is predicated on this finding.

Specifically, the present invention provides:
1) A golf ball comprising a core and a cover having an inner and an outer layer surrounding the core, the outer cover layer having a surface formed with a plurality of dimples, characterized in that
   a product of the Shore D hardness of said inner cover layer multiplied by the Shore D hardness of said outer cover layer and a proportion V_{R} (%) of the total of the volumes of dimple spaces each defined below a plane circumscribed by the dimple edge to the overall volume of a phantom sphere given on the assumption that the golf ball surface is free of dimples satisfy any one of the following combinations (1) to (5):
   (1) the product of Shore D hardnesses of inner and outer cover layers: 1,500 to less than 2,000
      V_{R}: 0.8 to 1.1%
   (2) the product of Shore D hardnesses of inner and outer cover layers: 2,000 to less than 2,500
      V_{R}: 0.75 to 1.05%
   (3) the product of Shore D hardnesses of inner and outer cover layers: 2,500 to less than 3,000
      V_{R}: 0.7 to 1%
   (4) the product of Shore D hardnesses of inner and outer cover layers: 3,000 to less than 3,500
      V_{R}: 0.65 to 0.95%
   (5) the product of Shore D hardnesses of inner and outer cover layers: 3,500 to 4,000
      V_{R}: 0.6 to 0.9%,
   and said dimples include at least three types of dimples which are different in at least one of a diameter, a depth, and a value V₀ which is the volume of one dimple space defined below a plane circumscribed by the dimple edge divided by the volume of a cylinder whose bottom is the plane and whose height is the maximum depth of the dimple from the bottom, characterised in that the golf ball is a multipiece solid golf ball comprising a solid core and the cover surrounds the solid core, wherein dimples of a first type have a diameter of 3.7 to 4.5 mm, a depth in the range 0.15 to 0.25 mm and a value V₀ of 0.38 to 0.55 wherein at least one of the diameter, the volume or the depth of the dimples of the first type are larger than the diameter, the volume or the depth respectively of any other type, and dimples of a second type have a diameter of 2.0 to 3.7 mm, a depth of 0.08 to 0.23 mm and a value V₀ of 0.38 to 55, wherein at least one of the diameter, the volume or the depth of the dimples of the second type are smaller than the diameter, the volume or the depth respectively of any other type.
2) The multi-piece solid golf ball of 1) wherein the solid core has a distortion of 2.6 to 6.5 mm under an applied load of 100 kg.
3) The multi-piece solid golf ball of 1) or 2) wherein both the hardnesses of the inner and outer cover layers are up to 63 in Shore D hardness.

### BRIEF DESCRIPTION OF THE DRAWINGS

FIG. 1 is a cross-sectional view of a dimple illustrating how to calculate a value V₀.
FIG. 2 is a perspective view of the dimple illustrating how to calculate a value V₀.
FIG. 3 is a cross-sectional view of the dimple illustrating how to calculate a value V₀.

Now the invention is described in more detail. The multi-piece solid golf ball of the invention is defined as comprising a solid core and a cover of two inner and outer layers surrounding the core, the outer cover layer having a surface formed with a plurality of dimples. When the range of the product of the Shore D hardnesses of the inner and outer cover layers is divided into sub-ranges, a dimple parameter can be specified in conjunction with each of the sub-ranges of the product for achieving optimization.

First, the solid core is described. The solid core may be formed of a well-known rubber composition. For example, it is prepared by mixing 1,4-cis-polybutadiene as a base with a well-known crosslinking agent, co-crosslinking agent, filler and so on in a roll mill, introducing a necessary amount of the composition into a solid core-shaping mold, and effecting vulcanization and heat molding. In this regard, the solid core may consist of a single layer or plural layers. In the practice of the invention, the solid core preferably undergoes a distortion or deformation of 2.6 to 6.5 mm, more preferably 2.7 to 6.3 mm, most preferably 2.8 to 6.0 mm under an applied load of 100 kg. A distortion of less than 2.6 mm (hard core) would exacerbate hitting feel. A distortion of more than 6.5 mm (soft core) would result in a ball with less restitution.

The golf ball of the invention is constructed by forming a cover of two (inner and outer) layer structure around the aforementioned solid core. The inner and outer layers may be formed of well-known cover stocks. Specifically, ionomer resins, thermoplastic polyester elastomers, and thermoplastic polyurethane elastomers may be used alone or in admixture of two or more. In the practice of the invention, cover stocks must be selected such that the product of the Shore D hardness of the inner cover layer multiplied by the Shore D hardness of the outer cover layer fall in the range of 1,500 to 4,000.

The Shore D hardnesses of the inner and outer cover layers may be identical with or different from each other insofar as the product of Shore D hardnesses falls in the range of 1,500 to 4,000. That is, the Shore D hardness of the inner cover layer may be substantially identical with the Shore D hardness of the outer cover layer. Alternatively, either one of the inner and outer cover layers may be softer or harder than the other. The hardness difference between the inner and outer cover layers may be appropriately determined.

Preferably the outer cover layer has a Shore D hardness of up to 63, more preferably 30 to 62, especially 35 to 61. With a Shore D hardness of more than 63, there is a risk that no spin is acquired due to a slip phenomenon between the cover and the club face. If the hardness of the outer cover layer is below 30, the ball would lose restitution.

On the other than, the inner cover layer preferably has a Shore D hardness of 28 to 68. Restitution would be lost with an inner cover layer hardness of less than 28 whereas hitting feel would be exacerbated by a hardness above 68.

The method for forming the inner and outer cover layers around the solid core is not critical and can be in accord with conventional ones. Included are a method of enclosing the solid core with a pair of hemispherical half cups of an inner cover layer composition, compression molding to join the cups to the core, placing it in an injection mold, and injecting an outer cover layer composition and another method of forming half cups from inner and outer cover layer compositions, respectively, mating them to form half cups of the two layer structure, enclosing the solid core with the half cups, and effecting compression molding.

The thus formed cover of the inner and outer layers may have any desired gage. Usually the inner cover layer has a gage of 0.5 to 3.0 mm, especially 1.0 to 2.5 mm, the outer cover layer has a gage of 0.5 to 2.5 mm, especially 1.0 to 2.3 mm, and the cover has a total gage of 1.0 to 5.5 mm, preferably 1.5 to 5.0 mm, especially 1.5 to 3.5 mm.

The multi-piece solid golf ball of the invention has a plurality of dimples formed in the outer cover layer. The dimples are formed such that when the product of the Shore D hardness of the inner cover layer multiplied by the Shore D hardness of the outer cover layer is in the range from 1,500 to 4,000, which is divided into sub-ranges, a factor V_{R} associated with the dimples, that is, a proportion V_{R} (%) of the total of the volumes of dimple spaces each defined below a plane circumscribed by the dimple edge to the overall volume of a phantom sphere given on the assumption that the golf ball surface is free of dimples has the following value.
(1) The product of Shore D hardnesses of inner and outer cover layers: 1,500 to less than 2,000
   V_{R}: 0.8 to 1.1%
(2) The product of Shore D hardnesses of inner and outer cover layers: 2,000 to less than 2,500
   V_{R}: 0.75 to 1.05%
(3) The product of Shore D hardnesses of inner and outer cover layers: 2,500 to less than 3,000
   V_{R}: 0.7 to 1%
(4) The product of Shore D hardnesses of inner and outer cover layers: 3,000 to less than 3,500
   V_{R}: 0.65 to 0.95%
(5) The product of Shore D hardnesses of inner and outer cover layers: 3,500 to 4,000
   V_{R}: 0.6 to 0.9%

More preferred ranges of V_{R} are given below.
(1) The product of Shore D hardnesses of inner and outer cover layers: 1,500 to less than 2,000
   V_{R}: 0.82 to 1.08%
(2) The product of Shore D hardnesses of inner and outer cover layers: 2,000 to less than 2,500
   V_{R}: 0.77 to 1.03%
(3) The product of Shore D hardnesses of inner and outer cover layers: 2,500 to less than 3,000
   V_{R}: 0.72 to 0.98%
(4) The product of Shore D hardnesses of inner and outer cover layers: 3,000 to less than 3,500
   V_{R}: 0.67 to 0.93%
(5) The product of Shore D hardnesses of inner and outer cover layers: 3,500 to 4,000
   V_{R}: 0.62 to 0.88%

With respect to the aforementioned range, if the value of V_{R} relative to the product of Shore D hardnesses deviates from the specified range, there result a prematurely falling trajectory and a reduced flight distance.

The value V_{R} is the sum of volumes Vp of dimple spaces defined in the golf ball surface to be described later and is calculated according to the following equation: ${V}_{R} = \frac{Vs}{\frac{4}{3} ⁢ π ⁢ {R}^{3}} \times 100$
wherein Vs is the sum of the volumes Vp of dimple spaces each below a circular plane circumscribed by the dimple edge and R is a ball radius.

It is noted that Vs in the above equation is represented by the following equation and V_{R} can be calculated by substituting the value of Vs into the above equation of V_{R}. $Vs = {N}_{1} ⁢ {Vp}_{1} + {N}_{2} ⁢ {Vp}_{2} + … + {N}_{n} ⁢ {Vp}_{n} = {\sum }_{i = 1}^{n} {N}_{i} ⁢ {Vp}_{i}$ Vp₁, Vp₂, ... Vpₙ represent the volumes of dimples of different dimensions and N₁, N₂, ... Nₙ represent the number of dimples having the volumes Vp₁, Vp₂, ... Vpₙ, respectively.

In addition to the above-mentioned requirement of V_{R} value, the dimples formed in the golf ball of the invention must further satisfy the requirement that there are included at least three types of dimples which are different in at least one of a diameter, a depth, and a value V₀ which is the volume of one dimple space defined below a plane circumscribed by the dimple edge divided by the volume of a cylinder whose bottom is the plane and whose height is the maximum depth of the dimple from the bottom. If the number of dimple types is less than 3, there arises the problem that the golf ball lofts too high or drops prematurely.

The value V₀ associated with the dimple requirement is described below. In the event that the planar shape of a dimple is circular, as shown in FIG. 1, a phantom sphere 2 having the ball diameter and another phantom sphere 3 having a diameter smaller by 0.16 mm than the ball diameter are drawn in conjunction with a dimple 1. The circumference of the other sphere 3 intersects with the dimple 1 at a point 4. A tangent 5 at intersection 4 intersects with the phantom sphere 2 at a point 6 while a series of intersections 6 define a dimple edge 7. The dimple edge 7 is so defined for the reason that otherwise, the exact position of the dimple edge cannot be determined because the actual edge of the dimple 1 is rounded. The dimple edge 7 circumscribes a plane 8 (circle having a diameter Dm). Then, the dimple space 9 located below the plane 8 as shown in FIGS. 2 and 3 has a volume Vp. A cylinder 10 whose bottom is the plane 8 and whose height is the maximum depth Dp of the dimple from the plane 8 has a volume Vq. The ratio V₀ of the dimple space volume Vp to the cylinder volume Vq is calculated. $Vp = {\int }_{0}^{\frac{Dm}{2}} ⁢ 2 ⁢ π ⁢ xy ⅆ x$ $Vq = \frac{πD ⁢ {m}^{2} ⁢ Dp}{4}$ ${V}_{0} = \frac{{V}_{p}}{{V}_{q}}$

In the event that the planar shape of a dimple is not circular, the maximum diameter or length of a dimple is determined, the plane projected shape of the dimple is assumed to be a circle having a diameter equal to this maximum diameter or length, and V₀ is calculated as above based on this assumption.

With respect to the dimples of different types according to the invention, dimples of the first type have a diameter of 3.7 to 4.5 mm, preferably 3.8 to 4.3 mm and a depth of 0.15 to 0.25 mm, preferably 0.155 to 0.23 mm, and their number is preferably 5 to 80%, especially 10 to 75% of the total dimple number. They are set to have a V₀ value of 0.38 to 0.55, and preferably V₀ is 0.4 to 0.52.

Among the dimples of different types, dimples of the second type have a diameter of 2.0 to 3.7 mm, preferably 2.4 to 3.6 mm and a depth of 0.08 to 0.23 mm, preferably 0.09 to 0.21 mm, and their number is preferably 1 to 40%, especially 2 to 30% of the total dimple number. They are set to have a V₀ value of 0.38 to 0.55, preferably 0.4 to 0.52.

The golf ball as a whole should preferably have a V₀ value of 0.38 to 0.55, more preferably 0.4 to 0.52, especially 0.42 to 0.5. A V₀ value of less than 0.38 is likely to lead to a non-long-lasting trajectory whereas a V₀ value of more than 0.55 is likely to lead to a high rise or a loft trajectory.

In the practice of the invention, the total number of dimples is not critical although usually 360 to 460 dimples especially 370 to 450 dimples are formed.

The golf ball of the invention can be used as tournament golf balls and constructed in accordance with the Rules of Golf to a diameter of not less than 42.67 mm and a weight of not greater than 45.93 grams.

The multi-piece solid golf ball of the invention has the advantages that various properties including spin, feeling and durability inherent to the multi-piece construction are further improved and an increased flight distance is expected due to the elimination of a high rise or dropping trajectory.

### EXAMPLE

Examples of the present invention are given below together with Comparative Examples by way of illustration and not by way of limitation.

### Examples and Comparative Examples

Solid cores having a diameter of 36.7 mm were prepared by mixing a rubber composition of the formulation shown in Table 1 in a roll mill and heat compression molding the composition at 155°C for 15 minutes.

Each solid core was enclosed with cover stocks shown in Table 2 in the order shown in Tables 4 and 5 to form an inner cover layer and an outer cover layer. The outer cover layer on the surface was formed with dimples shown in Tables 3, 4, and 5. Three-piece solid golf balls were obtained in this way.

The golf balls thus obtained were examined for flight distance and trajectory by the following tests. The results are shown in Tables 4 and 5.

### Flight performance

Using a swing robot by True Temper Co., the ball was hit with a driver at a head speed of 48 m/sec. (#W1/HS48) to measure a spin, carry and total distance

### Trajectory

Twelve golf balls of each example were hit under the same conditions as in the flight performance test to visually observe a trajectory.

**Table 1**

| Solid core composition (pbw) | I | II | III | IV |
|---|---|---|---|---|
| 1,4-polybutadiene (cis structure) | 100 | 100 | 100 | 100 |
| Zinc acrylate | 32 | 32 | 23 | 33 |
| Dicumyl peroxide | 1.2 | 1.2 | 1.2 | 1.2 |
| Antioxidant | 0.1 | 0.1 | 0.1 | 0.1 |
| Zinc oxide | 5 | 5 | 5 | 4 |
| Barium sulfate | 13.2 | 23.1 | 26.8 | 0 |
| Peptizer | 1 | 1 | 1 | 0 |

**Table 2**

| Cover stock (pbw) | A | B | C | D | E | F |
|---|---|---|---|---|---|---|
| Hytrel 4047 | 100 | - | - | - | - | - |
| Surlyn 8120 | - | 50 | - | 30 | - | - |
| Himilan 1557 | - | 50 | - | - | - | 50 |
| Himilan 1856 | - | - | 90 | - | - | - |
| NO825J | - | - | 10 | - | - | - |
| Himilan 1605 | - | - | - | 20 | - | 50 |
| Himilan 1706 | - | - | - | 50 | - | - |
| PANDEX T-7890 | - | - | - | - | 100 | - |

| | | | | | | |
|---|---|---|---|---|---|---|
| Hytrel 4047: Toray duPont K.K., polyester base thermoplastic elastomer NO825J: Mitsui duPont K.K., ethylene/methacrylic acid/methacrylate terpolymer (nuclel) Surlyn 8120: E. I. duPont, ionomer resin Himilan 1557: Mitsui duPont Polychemicals K.K., ionomer resin Himilan 1856: Mitsui duPont Polychemicals K.K., ionomer resin Himilan 1605: Mitsui duPont Polychemicals K.K., ionomer resin Himilan 1706: Mitsui duPont Polychemicals K.K., ionomer resin PANDEX T-7890: Dai-Nihon Ink Chemical Industry K.K., thermoplastic polyurethane elastomer | | | | | | |

Note that an appropriate amount of titanium dioxide was blended in resin compositions A to F.

**Table 3**

| Type | Diameter (mm) | Depth (mm) | V₀ | Number | V_{R} (%) |
|---|---|---|---|---|---|
| 1 | 4.100 | 0.195 | 0.440 | 32 | 0.89 |
| | 4.200 | 0.195 | 0.440 | 40 | |
| | 4.000 | 0.195 | 0.440 | 184 | |
| | 3.900 | 0.195 | 0.440 | 16 | |
| | 3.400 | 0.195 | 0.440 | 104 | |
| | 3.350 | 0.195 | 0.440 | 16 | |
| 2 | 4.100 | 0.210 | 0.450 | 32 | 0.86 |
| | 4.200 | 0.180 | 0.450 | 40 | |
| | 4.000 | 0.165 | 0.450 | 184 | |
| | 3.900 | 0.200 | 0.450 | 16 | |
| | 3.400 | 0.155 | 0.450 | 104 | |
| | 3.350 | 0.160 | 0.450 | 16 | |
| 3 | 3.850 | 0.160 | 0.500 | 288 | 0.80 |
| | 3.250 | 0.150 | 0.500 | 72 | |
| | 2.500 | 0.140 | 0.500 | 42 | |
| 4 | 3.850 | 0.175 | 0.525 | 288 | 0.93 |
| | 3.250 | 0.170 | 0.530 | 72 | |
| | 2.500 | 0.170 | 0.530 | 42 | |
| 5 | 4.000 | 0.160 | 0.480 | 114 | 0.77 |
| | 4.000 | 0.180 | 0.480 | 42 | |
| | 3.650 | 0.140 | 0.480 | 180 | |
| | 3.600 | 0.140 | 0.480 | 24 | |
| | 2.550 | 0.100 | 0.480 | 60 | |
| 6 | 3.900 | 0.150 | 0.470 | 240 | 0.66 |
| | 3.200 | 0.150 | 0.470 | 120 | |
| 7 | 3.850 | 0.170 | 0.465 | 340 | 1.04 |
| | 3.600 | 0.170 | 0.465 | 140 | |
| 8 | 3.850 | 0.185 | 0.460 | 340 | 1.12 |
| | 3.600 | 0.185 | 0.460 | 140 | |

**Table 4**

| | | E1 | E2 | E3 | E4 | E5 |
|---|---|---|---|---|---|---|
| Solid core | Composition | I | II | III | IV | III |
| | Hardness* (mm) | 3.0 | 3.0 | 4.5 | 2.8 | 4.5 |
| inner cover layer | Stock | A | C | D | A | B |
| | Shore D hardness | 40 | 49 | 55 | 40 | 58 |
| | Gage (mm) | 1.5 | 1.5 | 1.5 | 1.5 | 1.5 |
| Outer cover layer | Stock | B | D | B | E | F |
| | Shore D hardness | 58 | 55 | 58 | 42 | 60 |
| | Gage (mm) | 1.5 | 1.5 | 1.5 | 1.5 | 1.5 |
| Dimple type | | 1 | 2 | 3 | 4 | 5 |
| Inner layer Shore D x outer layer Shore D | | 2320 | 2695 | 3190 | 1680 | 3480 |
| V_{R} (%) | | 0.89 | 0.86 | 0.80 | 0.93 | 0.77 |
| #W1/HS48 | Spin (rpm) | 2530 | 2540 | 2450 | 2680 | 2250 |
| | Carry (m) | 225 | 229 | 228 | 228 | 227 |
| | Total (m) | 255 | 257 | 258 | 257 | 258 |
| Trajectory | | somewhat rising, long-lasting, relatively low trajectory | rising, similar to balata ball | liner-like, long-lasting, medium trajectory | rising, similar to balata ball | liner-like, long-lasting, medium trajectory |

| | | | | | | |
|---|---|---|---|---|---|---|
| * a distortion (mm) of the solid core under an applied load of 100 kg | | | | | | |

**Table 5**

| | | CE1 | CE2 | CE3 |
|---|---|---|---|---|
| Solid core | Composition | I | III | IV |
| | Hardness* (mm) | 3.0 | 4.5 | 2.8 |
| Inner cover layer | Stock | A | D | A |
| | Shore D hardness | 40 | 55 | 40 |
| | Gage (mm) | 1.5 | 1.5 | 1.5 |
| Outer cover layer | Stock | B | B | E |
| | Shore D hardness | 58 | 58 | 42 |
| | Gage (mm) | 1.5 | 1.5 | 1.5 |
| Dimple type | | 6 | 7 | 8 |
| Inner layer Shore D x outer layer Shore D | | 2320 | 3190 | 1680 |
| V_{R} (%) | | 0.73 | 1.04 | 1.12 |
| #W1/HS48 | Spin (rpm) | 2530 | 2450 | 2680 |
| | Carry (m) | 220 | 218 | 217 |
| | Total (m) | 247 | 243 | 245 |
| Trajectory | | liner-like, high | liner-like, low, dropping | liner-like, low, dropping |

| | | | | |
|---|---|---|---|---|
| * a distortion (mm) of the solid core under an applied load of 100 kg | | | | |

As seen from the results of Examples, the multi-piece solid golf balls of the invention exhibit a satisfactory trajectory and are excellent in all of spin, carry, and total flight distance.

In contrast, the multi-piece solid golf ball of Comparative Example 1 wherein V_{R} is below the specified range associated with the product of the Shore D hardnesses of the inner and outer cover layers was inferior in flight distance performance. The multi-piece solid golf balls of Comparative Examples 2 and 3 wherein V_{R} is above the specified range was inferior in flight distance performance and exhibited a dropping trajectory.

## Claims

1. A golf ball comprising a core and a cover having an inner and an outer layer surrounding the core, the outer cover layer having a surface formed with a plurality of dimples (1),
a product of the Shore D hardness of said inner cover layer multiplied by the Shore D hardness of said outer cover layer and a proportion V_{R} (%) of the total of the volumes of dimple spaces (1) each defined below a plane (8)circumscribed by the dimple edge (7) to the overall volume of a phantom sphere given on the assumption that the golf ball surface is free of dimples satisfy any one of the following combinations (1) to (5):
(1) the product of Shore D hardnesses of inner and outer cover layers: 1,500 to less than 2,000
V_{R}: 0.8 to 1.1%
(2) the product of Shore D hardnesses of inner and outer cover layers: 2,000 to less than 2,500
V_{R}: 0.75 to 1.05%
(3) the product of Shore D hardnesses of inner and outer cover layers: 2,500 to less than 3,000
V_{R}: 0.7 to 1%
(4) the product of Shore D hardnesses of inner and outer cover layers: 3,000 to less than 3,500
V_{R}: 0.65 to 0.95%
(5) the product of Shore D hardnesses of inner and outer cover layers: 3,500 to 4,000
V_{R}: 0.6 to 0.9%,
and said dimples (1)include at least three types of dimples (1) which are different in at least one of a diameter (Dm), a depth (Dp), and a value V₀ which is the volume of one dimple space defined below a plane (8) circumscribed by the dimple edge (7) divided by the volume of a cylinder (10) whose bottom is the plane (8) and whose height is the maximum depth (Dp) of the dimple (1) from the bottom, **characterised in that** the golf ball is a multipiece solid golf ball comprising a solid core and the cover surrounds the solid core, wherein dimples of a first type have a diameter of 3.7 to 4.5 mm, a depth in the range 0.15 to 0.25 mm and a value V₀ of 0.38 to 0.55, wherein at least one of the diameter, the volume or the depth of the dimples of the first type are larger than the diameter, the volume or the depth respectively of any other type, and dimples of a second type have a diameter of 2.0 to 3.7 mm, a depth of 0.08 to 0.23 mm and a value V₀ of 0.38 to 0.55, wherein at least one of the diameter, the volume or the depth of the dimples of the second type are smaller than the diameter, the volume or the depth respectively of any other type.

2. The multi-piece solid golf ball of claim 1 wherein the solid core has a distortion of 2.6 to 6.5 mm under an applied load of 100 kg.

3. The multi-piece solid golf ball of claim 1 or 2 wherein the hardnesses of both the inner and outer cover layers are 63 or less in Shore D hardness.

4. The multi-piece solid golf ball of claim 1, wherein the number of the dimples of the first type is 5 to 80% of the total dimple number and the number of the dimples of the second type is 1 to 40% of the total dimple number.

## Patentansprüche

1. Golfball umfassend einen Kern und eine Ummantelung mit einer inneren und einer äußeren, den Kern umgebenden Schicht, wobei die äußere Ummantelungsschicht eine Oberfläche hat, die von einer Mehrzahl von Vertiefungen (1) gebildet wird,
Produkt der Short D-Härte der inneren Ummantelungsschicht, die mit der Short D-Härte der äußeren Ummantelungsschicht multipliziert wird, und ein Mengenverhältnis V_{R} (%) der Gesamtheit der Volumen der Vertiefungsabstände (1), wobei jeder unterhalb einer Ebene (8) definiert ist, die durch den Vertiefungsrand (7) abgegrenzt wird, gegenüber dem Gesamtvolumen einer gegebenen Phantomsphäre, wenn man davon ausgeht, dass die Oberfläche des Golfballs frei von Vertiefungen ist, und jedweden der folgenden Kombinationen (1) bis (5) entspricht:
(1) Produkt von Shore D-Härten von inneren und äußeren Ummantelungsschichten: 1.500 bis weniger als 2.000
V_{R}: 0,8 bis 1,1%
(2) Produkt von Shore D-Härten von inneren und äußeren Ummantelungsschichten: 2.000 bis weniger als 2.500
V_{R}: 0,75 bis 1,05%
(3) Produkt von Shore D-Härten von inneren und äußeren Ummantelungsschichten: 2.500 bis weniger als 3.000
V_{R}: 0,7 bis 1%
(4) Produkt von Shore D-Härten von inneren und äußeren Ummantelungsschichten: 3.000 bis weniger als 3.500
V_{R}: 0,65 bis 0,95%
(5) Produkt von Shore D-Härten von inneren und äußeren Ummantelungsschichten: 3.500 bis 4.000
V_{R}: 0,6 bis 0,9%
und die Vertiefungen (1) schließen mindestens drei Arten von Vertiefungen (1) ein, die in mindestens einem der folgenden Parameter verschieden sind: einem Durchmesser (Dm), einer Tiefe (Dp), und einem Wert V₀, der das Volumen eines unterhalb einer Ebene (8) definierten Vertiefungsabstands darstellt, wobei die Ebene (8) durch den Vertiefungsrand (7) abgegrenzt wird, dividiert durch das Volumen eines Zylinders (10), dessen Boden die Ebene (8) ist und dessen Höhe die maximale Tiefe (Dp) der Vertiefung vom Boden aus ist, **dadurch gekennzeichnet, dass** der Golfball ein mehrteiliger fester Golfball ist, umfassend einen festen Kern und **dadurch**, dass die Ummantelung den festen Kern umgibt, wobei die Vertiefungen einer ersten Art einen Durchmesser von 3,7 bis 4,5 mm, eine Tiefe im Bereich von 0,15 bis 0,25 mm und einen Wert V₀ 0,38 bis 0,55 hat, wobei mindestens einer der folgenden Parameter: der Durchmesser, das Volumen oder die Tiefe der Vertiefungen der ersten Art größer als jeweils der Durchmesser, das Volumen oder die Tiefe jedweder anderen Art ist, und Vertiefungen einer zweiten Art einen Durchmesser von 2,0 bis 3,7 mm, eine Tiefe von 0,08 bis 0,23 mm und einen Wert V₀ von 0,38 bis 0,55 haben, wobei mindestens einer der folgenden Parameter: der Durchmesser, das Volumen oder die Tiefe der Vertiefungen der zweiten Art kleiner als jeweils der Durchmesser, das Volumen oder die Tiefe jedweder anderen Art ist.

2. Mehrteiliger fester Golfball nach Anspruch 1, wobei der fester Kern eine Verformung von 2,6 bis 6,5 mm unter einer angewandten Last von 100 kg aufweist.

3. Mehrteiliger fester Golfball nach Anspruch 1 oder 2, wobei die Härten der inneren und äußeren Ummantelungsschichten 63 oder weniger in der Short D-Härte betragen.

4. Mehrteiliger fester Golfball nach Anspruch 1, wobei die Zahl der Vertiefungen der ersten Art 5 bis 80% der Gesamtzahl der Vertiefungen beträgt und die Zahl der Vertiefungen der zweiten Art 1 bis 40% der Gesamtzahl der Vertiefungen beträgt.

## Revendications

1. Balle de golfe comprenant un noyau et un revêtement ayant une couche interne et une couche externe entourant le noyau, la couche de revêtement externe ayant une surface formée par une pluralité de fossettes (1),
produit de dureté Shore D de ladite couche de revêtement interne multiplié par la dureté de Shore D de ladite couche de revêtement externe et une proportion V_{R} (%) du total des volumes des espaces de fossettes (1) chacun défini en dessous d'un plan (8) circonscrit par le bord de la fossette (7) au volume hors-tout d'une sphère fantôme donnée en présupposant que le surface de la balle de golfe est exempte de fossettes, et satisfaisant l'une quelconque des combinaisons (1) à (5) suivantes:
(1) le produit des duretés Shore D des couches de revêtement interne et externe : 1.500 à moins de 2.000
V_{R} : 0,8 à 1,1 %
(2) le produit des duretés Shore D des couches de revêtement interne et externe : 2.000 à moins de 2.500
V_{R} : 0, 75 à 1,05%
(3) le produit des duretés Shore D des couches de revêtement interne et externe : 2.500 à moins de 3.000
V_{R} : 0,7 à 1%
(4) le produit des duretés Shore D des couches de revêtement interne et externe : 3.000 à moins de 3.500
V_{R} : 0,65 à 0,95%
(5) le produit des duretés Shore D des couches de revêtement interne et externe : 3.500 à 4.000
V_{R} : 0,6 à 0,9%
et lesdites fossettes (1) incluent au moins trois types de fossettes (1) qui sont différents dans au moins un des paramètres parmi le diamètre (Dm), la profondeur (Dp), et une valeur V₀ qui est le volume d'un espace de fossette défini en dessous d'un plan (8) circonscrit par le bord de la fossette (7) divisé par le volume d'un cylindre (10) dont le fond est le plan (8) et dont la hauteur est la profondeur maximale (Dp) de la fossette (1) à partir du fond, **caractérisé en ce que** la balle de golf est une balle de golf solide multipièce comprenant un noyau solide et **en ce que** le revêtement entoure le noyau solide, les fossettes d'un premier type ayant un diamètre de 3,7 à 4,5 mm, une profondeur allant de 0,15 à 0,25 et une valeur V₀ de 0,38 à 0,55, au moins un paramètre parmi le diamètre, le volume ou la profondeur des fossettes du premier type sont plus grands que le diamètre, le volume ou la profondeur respectivement de tout autre type, et des fossettes d'un deuxième type ont un diamètre de 2,0 à 3,7 mm, une profondeur de 0,08 à 0,23 mm et une valeur V₀ de 0,38 à 0,55, au moins un des paramètres parmi le diamètre, le volume ou la profondeur des fossettes du deuxième type est plus petit que le diamètre, le volume ou la profondeur, respectivement, de tout autre type.

2. Balle de golf solide multipièce selon le revendication 1, dans laquelle le noyau solide a une distorsion de 2,6 à 6,5 mm sous une charge appliquée de 100 kg.

3. Balle de golf solide multipièce selon la revendication 1 ou 2, dans laquelle les duretés des couches de revêtement interne et externe sont de 63 ou moins dans la dureté Shore D.

4. Balle de golf solide multipièce selon le revendication 1, dans laquelle le nombre de fossettes du premier type est de 5 à 80% du nombre total de fossettes et le nombre de fossettes du deuxième type est de 1 à 40% du nombre total de fossettes.
